

# UNITED STATES PATENT OFFICE.

GOTTLIEB REICHERT, OF COBB, WISCONSIN.

## IRONING-GLOSS.

No. 888,655.

Specification of Letters Patent.

Patented May 26, 1908.

Application filed January 2, 1908. Serial No. 409,012.

*To all whom it may concern:*

Be it known that I, GOTTLIEB REICHERT, a citizen of the United States, residing at Cobb, in the county of Iowa and State of Wisconsin, have invented a new and useful Ironing-Gloss, of which the following is a specification.

This invention relates to a compound for imparting a glossy and finished appearance 10 to ironed garments.

The object of the invention is to provide a compound of this character which may be easily applied, which will not injure the finest fabrics, which can be used either with starch, 15 or after starching has been completed, and which may readily be manufactured without the employment of special machinery for the purpose.

With the above and other objects in view, 20 as will appear as the nature of the invention is better understood, the same consists in the novel ironing gloss hereinafter described and claimed.

The compound consists of the following 25 ingredients by weight—water, sixty-four ounces, purified beef tallow, ten ounces, borax, eight ounces, paraffin, four ounces, white bees wax, ten ounces, white soap, one ounce.

The compound is prepared in the following manner: The water is heated to 212° 20 F., and the other ingredients are then added in sequence as follows—borax, tallow, paraffin, wax and soap. The heat is applied, accompanied by stirring until all of the elements are thoroughly commingled. While 35 it will generally be preferred to use boiling water in compounding the ingredients, cold water may be employed, the only effect being that it will take a longer time to prepare the compound. 40

I claim:

The herein described ironing gloss consisting of the following ingredients in the stated proportions, substantially, by weight—water, sixty four ounces, purified beef tallow, 45 ten ounces, borax, eight ounces, paraffin, four ounces, white bees wax, ten ounces, and white soap, one ounce.

In testimony that I claim the foregoing as my own, I have hereto affixed my signature 50 in the presence of two witnesses.

GOTTLIEB REICHERT.

Witnesses:

JOHN H. ROHDE,  
CLARA ROACH.